

Jan. 16, 1923.

1,442,730

L. P. OHLIGER ET AL.  
METHOD OF MOLDING.  
FILED APR. 10, 1919.



Fig. 2



Fig. 1

WITNESS:

Clara Holmes.

Ralph Munden

INVENTOR.

Lewis P. Ohliger.  
Albert A. Reid.

BY

Raymond H. Van Nest

ATTORNEY.

## UNITED STATES PATENT OFFICE.

LEWIS P. OHLIGER AND ALBERT R. REID, OF NIAGARA FALLS, NEW YORK, ASSIGNEES  
TO U. S. LIGHT & HEAT CORPORATION, OF NIAGARA FALLS, NEW YORK, A COR-  
PORATION OF NEW YORK.

## METHOD OF MOLDING.

Application filed April 10, 1919. Serial No. 288,966.

To all whom it may concern:

Be it known that we, LEWIS P. OHLIGER and ALBERT R. REID, citizens of the United States, residing at Niagara Falls, in the county of Niagara and State of New York, have invented new and useful Improvements in Methods of Molding, of which the following is a specification.

The present invention relates to methods 10 of molding.

More particularly the present invention relates to methods of molding metals or alloys which are readily fusible. Said invention is particularly applicable to molding 15 certain parts of storage battery cells and will be described in connection with the molding of the strap which is used in a storage battery cell to mechanically and electrically connect plates of like polarity.

20 An object of the present invention is to provide a method of molding which will produce a uniform product and in which any defects will be readily apparent.

A further object is to provide a method of 25 molding whereby solid members may be readily connected together in an integral structure.

30 A further object is to provide a simple and inexpensive method of connecting storage battery plates together by fusing the lugs thereof by pouring in contact with said lugs a metal or alloy at a temperature higher than the melting point of said lugs, whereby said lugs and said molten metal will solidify 35 into an integral structure.

Other objects will be apparent as the description proceeds.

Referring to the drawings:—

Fig. 1 is a perspective view representing 40 a plurality of plates of like polarity connected together by means of a strap.

Fig. 2 is a schematic view illustrating in bare outline a mold which may be used for carrying out the present invention.

45 The plates used in storage batteries commonly consist of an alloy of lead and antimony. The amount of antimony present materially affects the melting point of the alloy, an increase of antimony up to a certain percentage having the effect of decreasing the melting point. The fact that the difference in percentage of antimony 50 changes materially the melting point of the

alloy, is used in carrying out the present invention.

The mold illustrated in Fig. 2 is indicated by the numeral 1. Said mold is provided with a pocket 2 upon its upper side, which pocket 2 has communicating therewith the vertical hole 3. This hole 3 is shaped to 60 provide a mold for the post which is commonly provided on storage battery straps. The battery plates are indicated by the numeral 4, each having a lug 5. The battery plates 4 will be held by any preferred means, 65 so that the lugs 5 project into the pocket 2 on the upper side of the mold 1. A vertically mounted pin 6 is adapted to have longitudinal movement within the hole 3 and to operate to close the bottom end of said 70 hole. Said pin 6 will be operated by the lever 7 which may be biased by gravity to rest against the stop 8. It will be apparent without further description that when molten metal is poured into the pocket 2, it 75 will fill up the hole 3 above the pin 6 and will also fill the pocket 2. As will be explained, this molten metal will unite with the lugs and an integral structure will be provided, having the strap 8 and post 9. 80 The lever 7 may be raised, whereby to loosen the molded structure from the mold, whereby the group of plates with the strap and post may be readily removed.

The molten metal for pouring the strap 85 and the post 9 will be chosen as an alloy having a higher melting point than the alloy of the lugs 5. As indicated above, this difference in melting point may be readily had by varying the percentage of antimony. 90 The molten alloy at the temperature higher than the melting point of the lugs 5 will fuse said lugs, whereby said lugs will be an integral part of the strap 8 and post 9. The antimony lead will not oxidize readily 95 when heated only a few degrees above its melting point. Therefore, the molten alloy may be kept free from impurities, whereby a perfect union with the plate lugs will result. The present invention is to be distinguished from the process of molding straps to battery lugs by superheating lead to a point above the fusing temperature of the lugs and pouring it around the lugs, thereby fusing said lugs to provide an integral 100 structure. According to the present invention.

tion in which no superheating of the molten alloy is required, precautions to prevent oxidation may be minimized, without decreasing the quality of the mold.

5 The process described above has advantages that inspection is easy and certain. An objection to the commonly used puddling process of attaching the straps to the plate lugs is that the joints between the lugs 10 and the strap are flooded with molten metal, whereby a superficial union looks perfect. According to the present invention no such deceiving appearances are produced. Inasmuch as the molding may be accomplished 15 with the plate lugs extending downwardly, there is no danger of molten metal running along the sides of the plates, as sometimes happens in the puddling process. The straps and posts are perfectly straight, so 20 there is no breakage of cell covers or plates caused by hammering the strap or cover in assembling. No skilled labor is required and the danger of lead poisoning is very much lessened.

25 It is to be understood that the apparatus illustrated is merely diagrammatical and is used only for the purpose of simplifying the description. Any other type of apparatus may be used and various modifications 30 may be made in the process described, without departing from the invention. It is intended that the patent shall cover all modifications that fall within the scope of the invention as defined by the appended claims.

35 What we claim as new and desire to secure by Letters Patent of the United States, is—

1. The method of uniting battery plate lugs containing an alloy of lead and another metal, which consists in causing said 40 lugs to become immersed in a molten alloy of metals the same as the lugs but having different percentages of constituent metals, to give a higher melting point thereto.

2. The method of integrally uniting the lugs of battery plates, which lugs contain 45 an alloy of lead and antimony, which consists in causing said lugs while extending downwardly, to be immersed in molten metal, said molten metal comprising an alloy of lead and antimony, and having a 50 lower percentage of antimony than said lugs.

3. The method of integrally uniting a member to a battery element, which element comprises an alloy of lead and antimony, 55 which consists in pouring molten metal in contact with solid metal, said molten metal having a lower percentage of antimony than said solid metal.

4. The method of integrally uniting a 60 member to a battery element, which element comprises an alloy of lead and antimony, which consists in pouring molten metal in contact with solid metal, said molten metal having a lower percentage of antimony than 65 said solid metal, said molten metal being maintained prior to and during pouring at a temperature below that at which it oxidizes readily.

5. The method of uniting battery plate 70 lugs containing an alloy of lead and antimony, which consists in pouring in contact with said lugs a molten alloy having a lower percentage of antimony than said lugs.

6. The method of uniting battery plate 75 lugs containing an alloy of lead and antimony, which consists in pouring in contact with said lugs a molten alloy having a lower percentage of antimony than said lugs, said molten metal being maintained 80 prior to and during pouring at a temperature below that at which it oxidizes readily.

In witness whereof, we have hereunto subscribed our names.

LEWIS P. OHLIGER.  
ALBERT R. REID.